

# UNITED STATES PATENT OFFICE.

DAVID S. OLIPHANT, OF TORONTO, CANADA.

## PROCESS OF MARKING TEXTILE FABRICS.

SPECIFICATION forming part of Letters Patent No. 443,375, dated December 23, 1890.

Application filed April 11, 1890. Serial No. 347,528. (No specimens.)

*To all whom it may concern:*

Be it known that I, DAVID SEWELL OLIPHANT, of the city of Toronto, in the county of York, in the Province of Ontario, Canada, have invented a certain new and Improved Process of Marking Textile Fabrics, of which the following is a specification.

The object of the invention is to provide a process for indelibly marking textile fabrics; and it consists in the employment of certain materials in the manner hereinafter more particularly explained, and then definitely pointed out in the claim.

In carrying out my process I make use of a marking-fluid and a mordant. The marking-fluid is prepared as follows: I take three drams and thirty-six grains of chloride of aniline, five drams of water, three drams and thirty-six grains of mucilage, and one dram and forty-eight minims or drops of glycerine, and thoroughly mix together, shaking the same daily for about two weeks, when it is ready for use. The mordant is prepared as follows: Eight grains of bichromate of potash, one ounce of heavy mucilage, and three ounces of pure water are mixed together. This mordant is first applied to the fabric to

be marked by a brush or otherwise, and when the fabric is dry the desired marking is done with the marking-fluid by the use of a pen, 30 stencil, or any appropriate means. When the ink is dry, the mordant may be readily washed out in either hot or cold water.

I prefer that the mordant and ink or marking-fluid should both be prepared in substantially the above proportions, and care should be taken not to mix them together, as their mixture would make a fluid that would quickly fade and become thick and useless for writing. 40

What I claim as my invention is—

The within-described process of marking textile fabrics, the same consisting in applying thereto a solution composed of bichromate of potash, mucilage, and water, and, after 45 drying, writing upon the prepared fabric with an ink composed of chloride of aniline, water, mucilage, and glycerine, substantially as specified.

Toronto, February 18, 1890.

DAVID S. OLIPHANT.

In presence of—

HUSON W. M. MURRAY,  
F. G. A. WRIGHT.